

# UNITED STATES PATENT OFFICE.

JOHN SHAW, OF HINDMARSH, SOUTH AUSTRALIA.

## TAWING HIDES OR SKINS.

SPECIFICATION forming part of Letters Patent No. 286,491, dated October 9, 1883.

Application filed April 16, 1883. (No specimens.) Patented in England December 7, 1882. No. 5,836.

*To all whom it may concern:*

Be it known that I, JOHN SHAW, residing at Hindmarsh, near Adelaide, in the Colony of South Australia, have invented an Improvement in Tawing Hides or Skins, (for which provisional protection in Great Britain, No. 5,836, dated December 7, 1882, has been obtained,) of which the following is a specification.

For converting hides and skins into leather they are usually, after preliminary treatment, subjected to the action of tan or tannic products. I have found that by employing, instead of tan or its equivalents, carbolic acid or compounds of carbolic acid—such as sulpho-carbolic acid—a considerable saving of time and labor can be effected; and my invention consists in applying these substances, and, when desirable, along with suitable media for penetrating the hides or skins. Various penetrating media may be employed—such as water, glycerine, oils, spirits, organic acids, bisulphide of carbon; also solutions or preparations of alkalies, soap, sugar, or flour, or mixtures of these substances. These do not effect the converting action of the carbolic acid or its equivalent, but may be selected as they may be best suited to the character of the leather that is to be produced. The proportions of the substances used for the treatment of the hides or skins may be varied. The following examples will sufficiently inform persons skilled in the art of manufacturing leather as to the character of the treatment according to my invention.

After the hides and skins are prepared in the usual way for tanning I treat them as follows: For producing a hard heavy leather,

suitable for soles, machine-beltting, and such like uses, I soak them in a mixture made in about the proportions of ten gallons water, one pound soap, and three pints carbolic acid, and I add daily carbolic acid enough to keep up the strength of the mixture until the hides are found to be sufficiently treated. For producing the softer kinds of leather I first soak the hides or skins for one or two days in a mixture made in about the proportions of four parts oil to one part carbolic acid, and then for several hours I soak them in a mixture of about four parts bisulphide of carbon to one part carbolic acid.

Instead of carbolic acid, compounds thereof—such as sulpho-carbolic acid and analogues of carbolic acid—may be used in the way described; but I prefer to employ carbolic acid, as being generally less costly than such other substances.

Having thus described the nature of my invention and the best way I know of carrying it into practical operation, I claim—

The within-described process of tawing hides or skins, consisting in preparing the hides or skins in the usual way for tanning, then soaking them for a day or more in a mixture of carbolic acid, and afterward soaking them in a mixture of bisulphide of carbon and carbolic acid, as specified.

In testimony whereof I have signed my name to this specification, in the presence of two subscribing witnesses, this 8th day of February, 1883.

JOHN SHAW.

Witnesses:

J. K. HAYCRAFT,  
J. D. PHILLIPS.